# EUROPEAN PATENT SPECIFICATION

(11) **EP 3 901 370 B1**
(45) Date of publication and mention of the grant of the patent: **07.06.2023**
(21) Application number: 21168793.4
(22) Date of filing: 16.04.2021
(51) Int. Cl.: E01C 13/08

(54) **ARAGONITE BASED INFILL MATERIAL**
FÜLLMATERIAL AUF BASIS VON ARAGONIT
MATÉRIAU DE REMPLISSAGE À BASE D'ARAGONITE

(30) Priority: 21.04.2020 US 202063013126 P; 16.11.2020 US 202017099175
(43) Date of publication of application: 27.10.2021
(73) Proprietor: Dawson Holdings, LLC, Baton Rouge LA 70808 (US)
(72) Inventor: DAWSON, Charles, Baton Rouge, LA 70808 (US)
(74) Representative: J A Kemp LLP

(56) References cited:
- FR-A1- 2 932 196
- US-A1- 2003 092 531
- US-B2- 7 128 497
- ANONYMOUS: "Agricultural Uses", INTERNET CITATION, 29 May 2019 (2019-05-29), XP002802769, Retrieved from the Internet: URL:https://web.archive.org/web/2019052903 2257/http://www.calcean.com/agriculture/ [retrieved on 2021-04-21]

## Description

### I. Background

Various types of sports fields such as football, baseball and soccer fields, are increasingly being constructed using various artificial turf systems which have a natural grass texture, but also have greater longevity and less maintenance than natural turf systems. Generally, artificial turf is a synthetic turf system which includes a grass layer made of a plurality of pile-fibers and an infill composed of particles or chips distributed between the pile-fibers. In some cases, the infill material consists of granulated rubber chips or particles. However, such rubber particles have many disadvantages, include degrading in sunlight, becoming soft and sticky in warm Summer temperatures, and having an unpleasant odor. When such rubber chips are produced from recycled tires, there is the concern of embedded heavy metals being released and inhaled by persons using the sports fields.

Sand has also been used as an infill material. But sand has its own disadvantages, including concerns regarding players being placed at higher risk of silicosis from inhaling silica in the form of fine sand dust. An improve infill material which overcomes many of the disadvantages of prior art infill materials would be a welcome advancement in the art.

US 2003/092531 A1 discloses vertical to horizontal draining synthetic turf. US 7 128 497 B2 discloses a horizontally draining artificial turf system. FR 2 932 196 A1 discloses a synthetic and natural turf and method of installation. The following document discloses agricultural uses of aragonite: ANONYMOUS: "Agricultural Uses", INTERNET CITATION, 29 May 2019 (2019-05-29), Retrieved from the Internet: URL: https://web.archive.org/web/20190529032257/http://www.calcean.com/agriculture/ [retrieved on 2021-04-21].

### II. Summary of Selected Embodiments of the Invention

In accordance with the present invention, there are provided a method of constructing a sports field having the features of claim 1 and a sports field having the features of claim 2.

The steps of the method first comprise (a) placing a drainage base on a section of ground to be occupied by the sports field; then (b) placing a turf over the drainage base; and finally, (c) distributing an infill material over the artificial turf with a loading of between 2.4 and 39 kg/m² (0.5 and 8 lbs/ft²), wherein the infill material comprises at least 75% by weight orthorhombic CaCO₃.

Another embodiment not falling under the scope of the claims is constructing a play area by placing this infill material at a depth of at least 5 cm (2 inches) across the designated play area.

A further embodiment not falling under the scope of the claims is a bagged non-silica or low-silica play material comprised of (45 kg) 100 lbs or less of the infill material placed in a sealed flexible container.

### III. Brief Description of the Drawings

Figure 1 illustrates one embodiment of an artificial turf system with an underlying drainage structure.

### IV. Detailed Description of Selected Embodiments

One embodiment of the present invention is a method of constructing a sports field. Figure 1 suggests the basic components of the sports field 75, which is also referred to as artificial turf system 75. Turf system 75 generally includes a stabilization layer 76 (e.g., a concrete layer) positioned on a compacted soil base, i.e., compacted subgrade 78. A water impervious liner 79 is positioned between subgrade 78 and stabilization layer 76. Positioned on top of the stabilization layer 76 is a drainage and shock attenuation blanket or layer 80. While the drainage blanket 80 can be any one of a number of conventional drainage materials or fabrics, in the Figure 1 embodiment, drainage blanket 80 is a GeoFlo^{®}. drainage and shock attenuation blanket available for Global Synthetics Environmental, LLC of St. Gabriel, La. Typically, the drainage blanket 80 is not attached to the stabilization layer, but is comparatively free moving with respect to the stabilization layer. An artificial turf layer 82 is placed over the drainage blanket layer 80, but not rigidly attached thereto except at the edges. In a preferred embodiment, the artificial turf layer 82 may be a product such as GeoGreen^{®} replicated grass also available from Global Synthetics Environmental, LLC. The ends of drainage blanket and turf layers will be enclosed by the concrete border curb 87. Adjacent to the border curb 87 will be the drainage channel 84 filed with aggregate such as No. 57 stone. The perforated drainage pipe 85 will be positioned at the bottom of drainage channel 84. Typically, the subgrade 78 will be formed to have a grade line 90 with at least a 1/2% slope falling toward the border curb 87. Thus, rainfall on the turf system will be directed via drainage blanket 80 toward the drainage channel 84 and ultimately into drainage pipe 85. The drainage blanket 80, drainage channel 84, and drainage pipe 85 may be considered as part of a drainage base underlying the turf layer 82. The Figure 1 drainage base is only one example and many other conventional and future developed drainage structures which divert water filtering through the turf layer could be employed.

Typically, the turf layer 82 has a granular infill material 1 spread over and into the "grass" portion of the turf. Sand is one typical prior art infill material and provides a more natural feel under foot and helps hold the turf in place. However, embodiments of the present invention will employ an infill material 1, which in preferred embodiments, is an orthorhombic calcium carbonate (CaCO3). This mineral is more commonly referred to as Aragonite.

Aragonite is one of the three most common naturally occurring crystal forms of calcium carbonate, CaCO3 (the other forms being the minerals calcite and vaterite). It is formed by biological and physical processes, including precipitation from marine and freshwater environments. The crystal lattice of aragonite differs from that of calcite, resulting in a different crystal shape, an orthorhombic crystal system with acicular crystal. Repeated twinning results in pseudo-hexagonal forms. Aragonite may be columnar or fibrous, occasionally in branching stalactitic forms. Typical examples of orthorhombic CaCO3 are obtained from natural sources, but there could be examples of the material being artificial or man-made. One preferred variety of Aragonite is known as Oolitic Argonite because of its generally egg-shaped particles.

The infill material 1 need not be pure Aragonite and in some embodiments can be as low as 75% by weight Aragonite and 25% other filler materials, including sand if the application does not require a substantially silica-free infill material. However, there are many applications where it is desirable to have a substantially silica-free infill material. In those applications, silica will be less than about 5% by weight of the infill material and preferably, less than 1% by weight (and conceivably less than any percentage between 5 and 0.001). In most applications, the infill material will have an Aragonite content of between about 75% and 99.9% by weigh (e.g., "at least" some percentage between 75% and 99.9%) depending on application requirements. These weight percentages are for substantially dry infill material, i.e., a water content of less than 3% and more preferably, less than 1% by weight.

The distribution loading of the infill material (i.e., kg of infill material applied per square metre of turf area, or lbs of infill material applied per square foot of turf area) may vary between about 1.2 kg/m² (0.25 lbs/ft²) and about 49 kg/m² (10 lbs/ft²) for most turf applications (or any subrange in between). Longer and/or less dense yarn (the artificial "grass" blades) will suggest a heavier loading while shorter and/or more dense yarn will suggest a lighter loading. Nor is application of the infill material strictly limited to artificial turfs, but could have application to natural turfs or grass. Also, the infill material could have application in a play area as a substitute for sand, for example a child's sandbox or a "beach" volleyball court. In these applications, the infill material could be placed with a depth of anywhere between 5 cm and 30 cm (2" and 12"). A greater depth is possible, but typically is not necessary. In many embodiments, the play area is surrounded by a raised border to retain the infill material, e.g., boards, landscape timbers, or landscaping blocks. In certain embodiments, the play area is anywhere between 2.3 m² (25 ft²) and 230 m² (2500 ft²).

In many embodiments, the infill material will be sieved to have a size distribution within a 20/100 mesh ratio. In certain embodiments, this 20/100 mesh ratio means that no more than about 1% of the material remains on a 20 mesh screen and no more than 6% reaches the 100 mesh screen. In other embodiments, this 20/100 mesh ratio may mean that at least 85% of the sieved material remains within the 20/100 mesh range. In one particular embodiment, 0-5% passes 100 mesh, 10-20% is retained on 100 mesh, 38-48% is retained on 48 mesh, 18-28% is retained on 32 mesh, 12-22% is retained on 28 mesh, and at least 95% passes 20 mesh. The infill material will also typically have a crush rating of at least about 45 MPa (6.5 kpsi) to at least about 60 MPa (9 kpsi) (or any subrange in between). The crush rating is the load that may be placed on the material without producing 10% fines (fines being material passing through a 100 mesh screen). The specific gravity of the infill material (i.e., of individual grains of the material as opposed to its bulk density) will be at least 2.75, more preferably, at least 2.85, and most preferably, at least 2.9 (or at least any value between 2.75 and 3.0). The bulk density may range between 1.35 and 1.85 g/cm³ (or any subrange in between, e.g., 1.42 to 1.59). Similarly, preferred embodiments of the infill material will have a Mohs hardness of between 3 and 4.5 (or any subrange in between). In certain embodiments, the infill materials will have a "roundness" classification based upon the British-Adopted European Standard BS EN 14955:2005, Surfaces for Sports Areas, of either B1, C1, or C2, with the roundness most preferably being C1. The infill will have this roundness classification when at least 75% of the individual grains of the infill material meet this roundness classification (or alternatively, at least 85%, 90%, 95%, or 99%).

In certain embodiments, the infill material will be packaged as a bagged non-silica or low-silica play material, e.g., a substitute for sand. In such embodiments, the infill material will typically be placed in bags containing no more than 45 kg (100 lbs) of the infill material, and more preferably, bags of 23 kg (50 lbs), or 11 kg (25 lbs). In another embodiment, the infill material will be placed in a bag containing about 900 kg (1 ton) of infill material.

Many of the embodiments of the infill material described above have significant advantages over the prior art. The infill material is cradle to cradle in that it is a biomimetic approach to the design of infill systems which models natural processes, where materials are viewed as nutrients circulating in healthy, safe metabolisms. The infill materials are substantially renewable, non-toxic, silica-free, and contain no heavy metals or carcinogens. Moreover, Aragonite has the ability to bind with many heavy metals which may otherwise exist in the environment, thereby preventing metals from being ingested by persons coming into contact with the infill material.

The CaCO3 infill material absorbs water at a rate similar to or higher than sand and slowly releases the moisture through the evaporative process (the process of liquid water evaporating from a surface which decreases the surface's temperature), which in turn allows this infill material to have a cooling effect on the surface surrounding or under the material. This cooling effect arises from the latent heat property of water. Water can hold heat without changing temperature, i.e., latent heat. Water has the ability to absorb heat from other surfaces, thereby preventing the secondary surface temperatures from rising as much as they otherwise would with conventional infill materials. When water absorbs enough heat, it evaporates, or changes phase from a liquid form to a gas form. The gas phase then leaves the surface and takes the absorbed heat with it. The result of this reaction is a decreased amount of heat and thus, decreased temperature in the surfaces around the infill material.

This ability to reduce temperature increase of the turf system can be quantified by techniques such as FIFA Test Method 14 for determination of heat on artificial turf products. See FIFA Quality Programme-46-Handbook of Test Methods for Football Turf, October 2015 (V.3.1, 16.03.2020). Under this FIFA Test Method, an artificial turf system employing the CaCO3 infill material is rated as Category 1 using the following scale:

**Table 1 (21.5.2. Categorisation):**

| **Category** | **Temperature Range °C** |
|---|---|
| Category 1 | <50 |
| Category 1-2 | 50-54 |
| Category 2 | 55-59 |
| Category 2-3 | 60-65 |
| Category 3 | > 65 |

The hardness and roundness of the CaCO3 infill material also results in the infill material being less likely to be ground or reduce to very fine dust-like particles through sustained use as a sports field infill. A reduction in dust derived from the infill is not only more healthy for the sports field users, but also prevents the pores of the water-drainage layers beneath the turf layer from becoming clogged with the dust particles. Experimentation found that 20 mm of CaCO3 infill applied to a 40 mm artificial turf layer resulted in the following characteristics:

| **Characteristic** | **Value** | **Rating** |
|---|---|---|
| Ball rebound | 0.81 m dry and 0.87 m wet | FIFA Quality or Quality Pro range |
| Shock absorption | 58 % dry and 59 % wet | FIFA Quality Range |
| Deformation | 6.4 mm dry and 6.8 mm wet | FIFA Quality or Quality Pro range |
| Energy Restitution | 32 % dry and 3 7 % wet | Approximating natural turf |
| Rot Resistance | 49 Nm dry and 48 Nm wet | FIFA Quality Range |
| CFH | 1.4 m | meets the Rugby requirement |
| Gmax | 74 | |

It will be understood the invention is not limited to infill materials which have some or all or the above stated advantages. The term "about" as used herein will typically mean a numerical value which is approximate and whose small variation would not significantly affect the practice of the disclosed embodiments. Where a numerical limitation is used, unless indicated otherwise by the context, "about" means the numerical value can vary by +/-5%, +/-10%, or in certain embodiments +/-15%, or possibly as much as +/-20%. Similarly, the term "substantially" will typically mean at least 85% to 99% of the characteristic modified by the term. For example, "substantially all" will mean at least 85%, at least 90%, or at least 95%, etc.

## Claims

1. A method of constructing a sports field (75) comprising the steps of:
(a) placing a drainage base (80, 84, 85) on a section of ground to be occupied by the sports field (75);
(b) placing an artificial turf (82) over the drainage base (80, 84, 85); and
(c) distributing an infill material (1) over the artificial turf (82),
**characterized in that** the infill material (1) is distributed over the artificial turf (82) with a loading of between 2.4 and 39 kg/m² (0.5 and 8 lbs/ft²), and the infill material (1) comprises at least 75% by weight orthorhombic CaCO₃.

2. A sports field (75) comprising:
(a) a drainage base (80, 84, 85) on a section of ground to be occupied by the sports field (75);
(b) an artificial turf (82) placed over the drainage base (80, 84, 85); and
(c) an infill material (1) distributed over the artificial turf (82),
**characterized in that** the infill material (1) is distributed over the artificial turf (82) with a loading of between 2.4 and 39 kg/m² (0.5 and 8 lbs/ft²), and the infill material (1) comprises at least 75% by weight orthorhombic CaCO₃.

3. The method of claim 1 or the sports field (75) of claim 2, wherein the infill material (1) comprises at least 90% by weight orthorhombic CaCO₃.

4. The method or sports field (75) of any one of the preceding claims, wherein the infill material (1) has a size distribution within a 20/100 mesh ratio.

5. The method or sports field (75) of any one of the preceding claims, wherein the infill material (1) has a crush rating of at least 45 MPa (6.5 kpsi).

6. The method or sports field (75) of claim 5, wherein the infill material (1) has a crush rating of at least 52 MPa (7.5 kpsi).

7. The method or sports field (75) of any one of the preceding claims, wherein the infill material (1) has specific gravity of at least 2.75.

8. The method or sports field (75) of claim 7, wherein the infill material (1) has specific gravity of at least 2.85.

9. The method or sports field (75) of any one of the preceding claims, wherein the infill material (1) has a silica content of less than 10%.

10. The method or sports field (75) of claim 9, wherein the infill material (1) has a silica content of less than 5%.

11. The method or sports field (75) of any one of the preceding claims, wherein the infill material (1) has a Mohs hardness of between about 3.5 and about 4.

12. The method or sports field (75) of any one of the preceding claims, wherein the infill material (1) at least 95% of the grains of infill material (1) have a C1 roundness classification under the BS EN 14955:2005 standard.

13. The method or sports field (75) of any one of the preceding claims, wherein the drainage base comprises a drainage blanket (80).

14. The method or sports field (75) of claim 13, wherein the drainage base further comprises a drainage channel (84) and a perforated drainage pipe (85) positioned at the bottom of the drainage channel.

## Patentansprüche

1. Verfahren zum Anlegen eines Sportplatzes (75), das die Schritte umfasst:
(a) Platzieren einer Dränungsbasis (80, 84, 85) auf einem Bereich des Bodens, der von dem Sportplatz (75) eingenommen werden soll;
(b) Platzieren eines Kunstrasens (82) über der Dränungsbasis (80, 84, 85); und
(c) Verteilen eines Füllmaterials (1) über den Kunstrasen (82),
**dadurch gekennzeichnet, dass** das Füllmaterial (1) über den Kunstrasen (82) mit einer Belastung zwischen 2,4 und 39 kg/m² (0,5 und 8 lbs/ft²) verteilt wird, und das Füllmaterial (1) wenigstens 75 Gew.-% orthorhombisches CaCO₃ umfasst.

2. Sportplatz (75), umfassend:
(a) eine Dränungsbasis (80, 84, 85) auf einem Bereich des Bodens, der von dem Sportplatz (75) eingenommen werden soll;
(b) einen Kunstrasen (82), der über der Dränungsbasis (80, 84, 85) platziert wird; und
(c) ein Füllmaterial (1), das über den Kunstrasen (82) verteilt wird,
**dadurch gekennzeichnet, dass** das Füllmaterial (1) über den Kunstrasen (82) mit einer Belastung zwischen 2,4 und 39 kg/m² (0,5 und 8 lbs/ft²) verteilt wird, und das Füllmaterial (1) wenigstens 75 Gew.-% orthorhombisches CaCO₃ umfasst.

3. Verfahren nach Anspruch 1 oder Sportplatz (75) nach Anspruch 2, wobei das Füllmaterial (1) wenigstens 90 Gew.-% orthorhombisches CaCO₃ umfasst.

4. Verfahren oder Sportplatz (75) nach einem der vorhergehenden Ansprüche, wobei das Füllmaterial (1) eine Größenverteilung innerhalb eines 20/100-Maschenzahlverhältnisses aufweist.

5. Verfahren oder Sportplatz (75) nach einem der vorangehenden Ansprüche, wobei das Füllmaterial (1) eine Druckfestigkeit von wenigstens 45 MPa (6,5 kpsi) aufweist.

6. Verfahren oder Sportplatz (75) nach Anspruch 5, wobei das Füllmaterial (1) eine Druckfestigkeit von wenigstens 52 MPa (7,5 kpsi) aufweist.

7. Verfahren oder Sportplatz (75) nach einem der vorhergehenden Ansprüche, wobei das Füllmaterial (1) eine spezifische Gravitation von wenigstens 2,75 aufweist.

8. Verfahren oder Sportplatz (75) nach Anspruch 7, wobei das Füllmaterial (1) eine spezifische Gravitation von wenigstens 2,85 aufweist.

9. Verfahren oder Sportplatz (75) nach einem der vorhergehenden Ansprüche, wobei das Füllmaterial (1) einen Siliciumdioxidgehalt von weniger als 10 % aufweist.

10. Verfahren oder Sportplatz (75) nach Anspruch 9, wobei das Füllmaterial (1) einen Siliciumdioxidgehalt von weniger als 5 % aufweist.

11. Verfahren oder Sportplatz (75) nach einem der vorhergehenden Ansprüche, wobei das Füllmaterial (1) eine Mohs-Härte zwischen etwa 3,5 und etwa 4 aufweist.

12. Verfahren oder Sportplatz (75) nach einem der vorhergehenden Ansprüche, wobei das Füllmaterial (1) wenigstens 95 % der Körner des Füllmaterials (1) eine Rundheitsklassifizierung C1 gemäß der Norm BS EN 4955:2005 aufweisen.

13. Verfahren oder Sportplatz (75) nach einem der vorhergehenden Ansprüche, wobei die Dränungsbasis eine Dränungsmatte (80) umfasst.

14. Verfahren oder Sportplatz (75) nach Anspruch 13, wobei die Dränungsbasis ferner eine Dränungsrinne (84) und ein perforiertes Dränungsrohr (85) umfasst, das an dem Boden der Dränungsrinne angeordnet ist.

## Revendications

1. Procédé de construction d'un terrain de sport (75) comprenant les étapes consistant à :
(a) placer une base de drainage (80, 84, 85) sur une section de terrain devant être occupée par le terrain de sport (75) ;
(b) placer un gazon artificiel (82) sur la base de drainage (80, 84, 85) ; et
(c) répartir un matériau de remplissage (1) sur le gazon artificiel (82), **caractérisé en ce que** le matériau de remplissage (1) est réparti sur le gazon artificiel (82) avec une charge comprise entre 2,4 et 39 kg/m² (0,5 et 8 livres/pied²), et le matériau de remplissage (1) comprend au moins 75 % en poids de CaCO₃ orthorhombique.

2. Terrain de sport (75) comprenant :
(a) une base de drainage (80, 84, 85) sur une section de terrain devant être occupée par le terrain de sport (75) ;
(b) un gazon artificiel (82) placé sur la base de drainage (80, 84, 85) ; et
(c) un matériau de remplissage (1) réparti sur le gazon artificiel (82), **caractérisé en ce que** le matériau de remplissage (1) est réparti sur le gazon artificiel (82) avec une charge comprise entre 2,4 et 39 kg/m² (0,5 et 8 livres/pied²), et le matériau de remplissage (1) comprend au moins 75 % en poids de CaCO₃ orthorhombique.

3. Procédé selon la revendication 1 ou terrain de sport (75) selon la revendication 2, dans lequel le matériau de remplissage (1) comprend au moins 90 % en poids de CaCO₃ orthorhombique.

4. Procédé ou terrain de sport (75) selon l'une quelconque des revendications précédentes, dans lequel le matériau de remplissage (1) a une distribution de taille dans un rapport de maille de 20/100.

5. Procédé ou terrain de sport (75) selon l'une quelconque des revendications précédentes, dans lequel le matériau de remplissage (1) a un taux de résistance à la compression d'au moins 45 MPa (6,5 kpsi).

6. Procédé ou terrain de sport (75) selon la revendication 5, dans lequel le matériau de remplissage (1) a un taux de résistance à la compression d'au moins 52 MPa (7,5 kpsi).

7. Procédé ou terrain de sport (75) selon l'une quelconque des revendications précédentes, dans lequel le matériau de remplissage (1) a une densité d'au moins 2,75.

8. Procédé ou terrain de sport (75) selon la revendication 7, dans lequel le matériau de remplissage (1) a une densité d'au moins 2,85.

9. Procédé ou terrain de sport (75) selon l'une quelconque des revendications précédentes, dans lequel le matériau de remplissage (1) a une teneur en silice inférieure à 10 %.

10. Procédé ou terrain de sport (75) selon la revendication 9, dans lequel le matériau de remplissage (1) a une teneur en silice inférieure à 5 %.

11. Procédé ou terrain de sport (75) selon l'une quelconque des revendications précédentes, dans lequel le matériau de remplissage (1) a une dureté Mohs comprise entre environ 3,5 et environ 4.

12. Procédé ou terrain de sport (75) selon l'une quelconque des revendications précédentes, dans lequel dans le matériau de remplissage (1) au moins 95 % des grains du matériau de remplissage (1) ont une classification d'arrondi C1 selon la norme BS EN 14955:2005.

13. Procédé ou terrain de sport (75) selon l'une quelconque des revendications précédentes, dans lequel la base de drainage comprend une nappe de drainage (80).

14. Procédé ou terrain de sport (75) selon la revendication 13, dans lequel la base de drainage comprend en outre un canal de drainage (84) et un tuyau de drainage perforé (85) positionné au fond du canal de drainage.
